

# UNITED STATES PATENT OFFICE.

ROBERT SUCHY, OF BITTERFELD, GERMANY, ASSIGNOR TO CHEMISCHE FABRIK GRIESHEIM ELECTRON, OF FRANKFORT-ON-THE-MAIN, GERMANY, A CORPORATION OF GERMANY.

## MANUFACTURE OF CHROMIC ACID.

No. 841,278.

Specification of Letters Patent.

Patented Jan. 15, 1907.

Application filed November 9, 1906. Serial No. 342,759.

*To all whom it may concern:*

Be it known that I, ROBERT SUCHY, a subject of the Emperor of Austria-Hungary, residing at Bitterfeld, Germany, have invented 5 certain new and useful Improvements in the Manufacture of Chromic Acid, of which the following is a specification.

This invention relates to the extraction of chromic acid from alkali chromates, alkali bichromates, and chromic acid containing sulfuric acid. Chromic acid has already been extracted from the said compounds by converting the bodies combined with the chromic acid into bisulfate; but the difficulty experienced in obtaining chromic acid by this means has been the separation of the chromic acid from the bisulfate, which has been a very troublesome and lengthy operation.

20 The object of this invention is to effect this separation in a simple manner and in a short time and with the use of very simple apparatus. The mixture of chromic acid and bisulfate is in accordance with this invention heated to the melting-point, this resulting in the formation of two fluids that are not miscible with each other and can therefore be easily separated from each other by mechanical means.

25 The invention may, for example, be carried out as follows: In any suitable vessel one hundred kilograms of sodium bichromate coarsely powdered are mixed with sixty-seven kilograms of sulfuric acid of 65.5° Baumé and heated while being stirred. Water is first evaporated, the mass becoming hard and pulverulent and on being further heated becomes a pulp or paste of molten bisulfate and solid 30 chromic acid. The temperature is then

raised until all the solid portions are melted, and the mass is allowed to cool down to 150° centigrade. The bisulfate and the chromic acid will then have separated, and the bisulfate is removed in any usual manner. The 45 remaining chromic acid is deprived by mechanical means of the bisulfate adhering to it and broken into pieces which do not contain more than from one and one-half to two per cent. of bisulfate.

50 When chromic acid is to be obtained from potassium bichromate, the process followed is similar. In obtaining chromic acid from its mixture with sulfuric acid the sulfuric acid is converted into bisulfate by means of 55 an alkali salt.

55 By the process according to this invention it is possible in a single operation to isolate the chromic acid in a high state of purity, whereas hitherto from three to four operations have been needed and yet the chromic acid has still been very impure owing to the presence of sulfuric acid.

I claim—

60 The herein-described process of manufacturing chromic acid which consists in mixing a chromate with sulfuric acid, heating the mixture whereby chromic acid and a bisulfate are formed and water evaporated, then fusing the mixture by heat and separating 65 the two fused superposed layers, substantially as described.

65 In testimony whereof I have signed my name to this specification in the presence of two subscribing witnesses.

ROBERT SUCHY.

Witnesses:

ERNST BORSBACH,  
AUGUST URICH.